

# UNITED STATES PATENT OFFICE.

JAMES M. SKINNER, OF PHILADELPHIA, PENNSYLVANIA, ASSIGNOR TO PHILADELPHIA STORAGE BATTERY COMPANY, OF PHILADELPHIA, PENNSYLVANIA, A CORPORATION OF PENNSYLVANIA.

## BATTERY-SEPARATOR AND PROCESS OF MAKING THE SAME.

1,130,640.

Specification of Letters Patent.

Patented Mar. 2, 1915.

No Drawing.

Application filed May 13, 1914. Serial No. 838,406.

*To all whom it may concern:*

Be it known that I, JAMES M. SKINNER, a citizen of the United States, residing in Philadelphia, Pennsylvania, have invented a certain Improvement in Battery-Separators and Processes of Making the Same, of which the following is a specification.

One object of my invention is to provide a relatively simple and inexpensive method 10 of treating sheets of wood to fit them for use as separators for the plates of secondary or storage batteries, the process being such that the separators produced possess in a high degree the qualities required of them; 15 *i. e.*, their internal resistance is low, their strength under working conditions in a battery is high, and they contain nothing which under ordinary conditions will injuriously act upon the materials of which the battery 20 plates are composed.

My invention also contemplates the provision of a battery separator having the above characteristics.

I have discovered that of the ordinary 25 woods available for use as battery separators, certain of them, such as white pine, Douglas fir, and the common species of cedar, possess to a high degree certain of the qualities desired, for they contain practically negligible amounts of material which 30 might injure the positive plates, such as acetic acid forming materials. They have, however, the objection that their internal resistance is relatively high. As a result of 35 my experiments, I have found that the presence of the small quantity of acetic acid forming compounds in the white pine and other wood separators hereinafter specified is beneficial to the negative battery plates 40 rather than harmful, so that in preparing the wood for use as separators in sheet or other form I subject it to a treatment which, while having practically no effect upon these compounds, serves to materially lower 45 its internal resistance. Further, the treatment does not remove lignone to an injuri-

ous extent, and consequently, the wood of the finished product is left structurally strong.

In carrying out my process I boil the 50 properly formed bodies of wood in water, preferably at atmospheric pressure, for a period of from 24 to 48 hours, more or less, although, in some cases, I may boil them in water under pressure up to 80 pounds to 55 the square inch for a period of from five to ten hours, although this time will vary with the wood and the pressure employed. Again, I may obtain the desired result by subjecting the wood to the action of steam under 60 pressure for a period of twelve hours, more or less. By any of the above described methods of treatment there is removed from the wood a sufficient amount of its resinous and possibly other insulating constituents, 65 with such a swelling and softening, as will lower its internal resistance to such an extent as to fit it for use as a battery separator. At the same time, the acetic acid forming compounds remain practically unaffected. I 70 have also found that the internal resistance of the wood may be lowered to the desired point without removing the acetic acid forming compounds, by treating it with a solvent other than water which removes only 75 the resinous constituents, and if alcohol be the substance employed, I immerse the wood in a body of this liquid, which may be heated to a temperature slightly below its boiling point, for such a length of time as is 80 necessary to attain the desired end. Obviously, the solvent may be employed under pressure in a closed vessel, as might be advisable in some cases.

I claim:—

1. The process of preparing battery separators which consists in shaping pieces of the wood of coniferous trees into the form of separators; and boiling said wood in water for a period equivalent to from 24 to 48 90 hours boiling in water at atmospheric pressure.

2. The process of preparing battery separators which consists in boiling the wood of coniferous trees in water for a period of from 24 to 48 hours.
5. 3. A battery separator produced by the herein described process which consists of coniferous wood containing a relatively small percentage of acetic acid forming compounds and including such an amount of

insulating compounds that its resistance is 10 relatively low.

In testimony whereof, I have signed my name to this specification, in the presence of two subscribing witnesses.

JAMES M. SKINNER.

Witnesses:

WILLIAM E. BRADLEY,  
Wm. A. BARR.